

(No Model.)

3 Sheets—Sheet 1.

J. WILLIAMS.

PROCESS OF PRODUCING CELLULOSE FILMS.

No. 444,515.

Patented Jan. 13, 1891.

Fig. 1.



Witnesses.

Battus de Long.  
C. W. Barkee

Inventor.  
James Williams,  
By his Atty.  
Baldon, Garrison & Night.

(No Model.)

3 Sheets—Sheet 2.

J. WILLIAMS.

PROCESS OF PRODUCING CELLULOSE FILMS.

No. 444,515.

Patented Jan. 13, 1891.



Witnesses.

Baltus D'Long.  
L. M. Brooke.

Inventor.

James Williams.  
By his Atty's.

Baldwin, Davidson & Wright.

(No Model.)

3 Sheets—Sheet 3.

J. WILLIAMS.

PROCESS OF PRODUCING CELLULOSE FILMS.

No. 444,515.

Patented Jan. 13, 1891.

*Fig. 3.*



Witnesses.

Baltus D. Long.

C. M. Brooke.

Inventor.  
James Williams.  
By his Atty.

*Baldwin, Dandurand & Night.*

# UNITED STATES PATENT OFFICE.

JAMES WILLIAMS, OF WILLESDEN JUNCTION, ENGLAND, ASSIGNOR TO THE PATENT WATERPROOF PAPER AND CANVAS COMPANY, LIMITED, OF SAME PLACE.

## PROCESS OF PRODUCING CELLULOSE FILMS.

SPECIFICATION forming part of Letters Patent No. 444,515, dated January 13, 1891.

Application filed January 16, 1890. Serial No. 337,108. (No specimens.)

*To all whom it may concern:*

Be it known that I, JAMES WILLIAMS, chemist, a subject of the Queen of Great Britain, residing at Willesden Paper Works, Willesden Junction, in the county of Middlesex, England, have invented certain new and useful Improvements in Processes of Producing Cellulose Films, of which the following is a specification.

- 10 The object of my invention is to produce an amorphous or structureless film upon the surface of paper or other suitable fibrous fabric or material, which is thus materially strengthened; and may be used for a great variety of purposes in the arts. A fabric having such a surface, for instance, may be used as a substitute for the albumenized paper now in common use for photographic purposes; or the unchanged portion of the fabric 15 may be separated from the cellulose film, which latter, being capable of resisting the action of water, steam, weak acids, and most solids, may be used for a great variety of purposes.
- 20 I produce this film by applying a solvent to the surface of the fabric and afterward eliminating the solvent from the film. I preferably apply the solvent to one surface only of the fabric, leaving the other surface unaltered, in contradistinction to the old way of dipping the fabric in the solvent, as such unaltered surface imparts strength to the sheet or fabric, so that it is easier to manipulate it both during and after the process of manufacture.
- 25
- 30
- 35

I prefer to proceed as follows in carrying out my invention: I first prepare a bath of strong cuprammonium hydro-oxide solution, which must be of the utmost possible purity, and I find it convenient to use from 1.5 to 2.5 per cent. of metallic copper, according to the degree of brilliancy required. I apply this bath to one side of the fabric, preferably by floating its surface thereon, care being taken that one side only of the fabric comes in contact with the solution, by which means I convert such surface into an amorphous, structureless, or approximately structureless film of cellulose, which is combined at this stage

with the oxide of copper, ammonia, and water. 50 The fabric is then, with as little exposure to the air as possible consistent with the setting of the film, exposed to heat, which is applied first to the unchanged surface of the fabric to expel the ammonia and water from the 55 deposited film. The fabric thus treated has a green tint, due to the copper hydrate contained in the deposited film. To remove this hydrate, and thus render the fabric suitable for photographic purposes, I apply a weak 60 acid thereto—such as sulphuric acid—which dissolves out the copper without affecting the glazed surface of the film. I prefer several consecutive applications of weak acid, as above described. The fabric is then washed 65 and dried, and is ready for use.

I separate the film from the unchanged fabric, when desired, by soaking the latter in water in well-known ways, so as to soften it, and thus render it readily removable. 70

The accompanying drawings represent a vertical longitudinal section through a convenient apparatus for carrying out my invention, the three sheets of drawings representing different portions, which when placed 75 end to end constitute the complete apparatus, of which—

Figure 1 shows the delivery end; Fig. 2, the central portion, and Fig. 3 the feed end, the fabric under treatment passing from 80 right to left.

The sheet or web of fabric passes from a roll A, between feed-rollers B, over the surface of a bath C of cuprammonium solution, the lower surface of the fabric being drawn 85 along in contact with the upper surface of the bath. The fabric then passes around a small guide-roller d and over leading-drums D D, upon which the dry surface of the fabric rests. Thence it passes round steam-heated 90 cylinders E' E<sup>2</sup>, with the first of which the dry side comes in contact in order to set the film and prevent its adhesion to the second cylinder E<sup>2</sup>, with which the film or treated side is kept in contact by an endless belt F, 95 traversing suitable rollers, as usual. If not sufficiently dry, the fabric may then pass around a third heated cylinder E<sup>3</sup>.

The whole apparatus is driven by endless belts in well-known ways to secure uniformity of speed and maintain the necessary slackness throughout, or, in other words, to avoid undue tension on the fabric.

When it is desired to render the film colorless, the fabric on which it has been formed, as above described, is passed through consecutive baths N N of weak acid, passing there-  
10 through under partially-submerged rollers O O and around rollers P between each bath. The fabric then traverses rollers in a water bath Q, thence over a revolving drum R into other water baths S, in which it is wholly sub-  
15 merged until free of all injurious impurities. The fabric is then taken by a third revolving drum R<sup>2</sup>, which need not be heated, around a series of cylinders T T, similar to those al-  
ready described, and heated in well-known  
20 ways, which gradually dry the fabric. The film thus treated, as hereinbefore remarked, is capable of withstanding the action of wa-  
ter, steam, weak acids, and alkalies, as well as ordinary solvents. This property enables  
25 me to remove the unchanged portion of the fabric, leaving only the film of cellulose.

Preferably I remove the unchanged portion of the fabric by washing the fabric in water with an ordinary or a rotary scrubbing-brush,  
30 but of course analogous means may be em-  
ployed.

Having thus fully described my improve-  
ments in the art of producing cellulose films,  
what I claim therein as new and as of my  
35 invention is—

1. The process hereinbefore described of exposing the fabric to the action of cupram-

monium hydro-oxide to form a film thereon, drying it to remove the ammonia, and then subjecting the fabric to the action of acid to 40 eliminate the copper.

2. The process hereinbefore described of floating the fabric upon the surface of a solvent, such as cuprammonium hydro-oxide, applying heat to the fabric, passing it suc-  
cessively through diluted acid and through  
water, and again drying it.

3. The process hereinbefore described of exposing the fabric to the action of the solvent, eliminating the solvent, and then remov-  
ing the unchanged portion of the fabric from 50 the amorphous film produced by the action  
of the solvent.

4. The process hereinbefore described of exposing the fabric to the action of cupram-  
monium hydro-oxide to form an amorphous  
55 film of cellulose thereon, then removing the  
ammonia by drying and the copper by acid,  
and afterward removing the unchanged portion  
of the fabric.

5. The process hereinbefore described of floating the fabric upon the surface of a solvent, such as cuprammonium hydro-oxide, to  
form an amorphous film of cellulose thereon,  
heating the fabric, subjecting it successively  
60 to the action of acid and to the action of wa-  
ter, again drying it, and afterward washing  
off the unchanged portion of the fabric.

JAMES WILLIAMS.

Witnesses:

JNO. H. WHITEHEAD,  
24 Southampton Buildings, London, W. C.

THOS. LAKE,

28 Southampton Buildings, London, W. C.